

## UNITED STATES PATENT OFFICE

2,611,727

BRAKE LINING AND METHOD OF MAKING  
SAME

Julius E. Underwood and Alfred Hirsch, Painesville, Ohio, assignors to Diamond Alkali Company, Cleveland, Ohio, a corporation of Delaware

No Drawing. Application October 20, 1949,  
Serial No. 122,582

10 Claims. (Cl. 154—81)

1

This invention relates to compositions of matter comprising siloxanes, and more particularly relates to compositions of matter comprising siloxanes and organic and inorganic additives which render the compositions especially suitable as friction elements, such as clutch facings, brake linings, and the like. The term "friction element," as used herein, is intended to mean a frictional energy absorbing member of an energy transfer mechanism for accelerating or decelerating motion in a mechanical system.

It has heretofore been broadly suggested that siloxanes, particularly the resinous siloxanes, are suitable as bonding materials in friction element compositions, principally because of their oil, grease, and heat resistance. Investigation has shown, however, that not all or even many of the various types of resinous siloxanes are suitable for such purposes, especially since much more than mere oil, grease, and heat resistance is required of the bonding material in a friction element. Moreover, it has been found by investigation that the effectiveness of even the most suitable siloxane materials in such compositions is affected in large part by the additives admixed therewith.

It is one of the objects of the present invention to provide commercially acceptable siloxane-containing friction element compositions.

Another object of the invention is to provide siloxane-containing friction element compositions of relatively simple formulation.

A further object of the invention is to provide siloxane-containing friction element compositions which have a low rate of wear and have a relatively high and constant coefficient of friction at high temperatures of the order of 600° to 1400° F.

The present invention is directed to compositions of matter, the principal ingredients of which include a cohydrolyzate of a mixture of 10-30 mol per cent of an ethyl silicon trihalide and 70-90 mol per cent of a phenyl silicon trihalide, suitably about 20 mol per cent of the former and 80 mol per cent of the latter, a physical mixture of lead sulfate and lead monoxide, and asbestos either in the form of fibers or in the form of a web, such as paper or cloth.

The mixtures of phenyl and ethyl silicon trihalides from which the cohydrolyzates used as bonding agents in the compositions of the present invention are derived may be obtained from any of the several phenyl or ethyl silicon trihalides but are preferably mixtures of phenyl and ethyl silicon trichlorides, since these latter compounds are somewhat more economically produced than

the other halide derivatives, particularly the phenyl and ethyl silicon tribromides or triiodides, and are more amenable to hydrolysis than the phenyl and ethyl silicon trifluorides. The cohydrolyzate of a mixture of these two compounds in the proportions stated is readily obtained by methods well known in the art, such as by combining the desired molar proportion of each of the preferred organosilicon chlorides in a suitable non-aqueous solvent and adding the solution of the mixture to an aqueous medium, which may contain in addition to the water therein, other organic or inorganic materials which tend to control the rate of the hydrolysis reaction. The co-hydrolyzate of the mixture of organosilicon trihalides may then be separated from the hydrolysis reaction mass in solution by ordinary gravity separation of the aqueous and non-aqueous phases. The co-hydrolyzate solution, or the resinous co-hydrolyzate obtained by evaporation of the solvent therefrom, may be used in compounding the compositions of the present invention. The amount of co-hydrolyzate to be employed in these compositions may be varied over a wide range and is between about 5% to 25% of the total weight of a composition, preferably within the range of 10% to 20% of the total weight of a composition. The particular sequence of steps employed in each of these techniques will be described more fully herein-after.

The physical mixture of lead sulfate and lead oxide employed in the compositions of the present invention is obtained by combining finely divided lead sulfate and finely divided lead oxide in suitable proportions. The fineness of the particles of these compounds is suitably of the order of 100-300 mesh, preferably of the order of 200-300 mesh. The compounds may be mixed in molar ratios of  $PbSO_4:PbO$  within the range of 0.4-1.1:1, preferably, however, within the range of 0.8-1.0:1. The mixture of  $PbSO_4$  and  $PbO$  is advantageously used in amounts ranging from 25% to 60% of the total weight of the compositions.

Asbestos is employed in the compositions of the present invention in amounts ranging from 20% to 75% by weight, either in the form of loose fibers or as webs, such as asbestos paper or cloth. Asbestos in either of these forms increases the tensile strength of molded articles obtained from these compositions and, in addition, provides a friction element composition of superior wear resistance and friction properties. Commercial grades of fibrous asbestos of uniform fiber length

such that none is retained on a screen having 0.5" openings, approximately 75% is retained on a 12 mesh screen, and the remaining 25% passing the 12 mesh screen is retained on a 16 mesh screen, are especially suitable in the compositions of the present invention when used in amounts ranging from 20% to 50% by weight. A commercial grade representative of this type is manufactured by the Johns-Manville Company and available as their grade "5-K." In addition, it has been found that webs of asbestos fibers, such as asbestos paper or woven asbestos cloth, generally ranging from 50% to 75% of the total weight of the compositions, further increase the tenacity and improve the friction properties of molded articles obtained from the compositions of the present invention. For example, it has been found that when asbestos webs, impregnated with a dispersion of the combination comprising a co-hydrolyzate of phenyl and ethyl silicon trihalides, and a mixture of lead sulfate and lead oxide in the molar proportions given above, are compressed under a pressure of approximately 4000 pounds per square inch, there results a molded article having a very low wear rate and a relatively high and constant coefficient of friction at high temperatures.

Small amounts, of the order of 2% to 10% of the total weight of the compositions, of heat resistant synthetic elastomeric polymers and copolymers, for example, copolymers of the butadiene-acrylonitrile type which are commercially available under the trade-name "Hycar," from the B. F. Goodrich Company, may be included in the compositions of the present invention and such elastomeric polymers and copolymers apparently function as plasticizers for the siloxane component of the compositions, thereby decreasing the brittleness of the siloxane binder and increasing the tenacity of the molded compositions.

Graphite may also be incorporated, if desired, particularly when the compositions are to be molded into friction elements. The amount of graphite, when so used, is preferably of the order of 1% to 5% of the total weight of the compositions.

In order that those skilled in the art may better understand the nature of the compositions of the present invention and in what manner the same may be obtained, the following specific examples are offered. For consistency in comparing the compositions of the several examples, a cohydrolyzate of 20 mol per cent of ethyl silicon trichloride and 80 mol per cent of phenyl silicon trichloride is used throughout as the siloxane binding material.

#### EXAMPLE 1

##### *Formulation*

442 parts of lead monoxide (approximately 300 mesh).

216 parts of fibrous asbestos (none retained on a screen having 0.5" openings, 75% retained on a 12 mesh screen, and 25% retained on a 16 mesh screen).

260 parts of a 61.5% solution in isopropyl ether of the co-hydrolyzate of 80 mol per cent of phenyl silicon trichloride and 20 mol per cent of ethyl silicon trichloride, containing 1.6 parts of triethanolamine (condensation catalyst for the organo-silicon trihalide co-hydrolyzate).

##### *Procedure*

The lead monoxide and asbestos are placed in a "Day" mixer (having eccentric contra-rotating masticating members), having a mixing chamber

which is jacketed for temperature control by means of steam and/or water. These dry materials are blended in the mixer at room temperature until a substantially uniform mix has been obtained. The solution of the organo-silicon halide co-hydrolyzate is added to the thoroughly blended combination of lead monoxide and asbestos and the entire mass mixed until substantial uniformity is obtained, after which the solvent is evaporated from the mass by admitting steam to the mixing chamber jacket. After substantially all of the solvent has been evaporated, a pulverulent mass of the mixture is obtained and removed from the mixing chamber. The substantially dry coherent particles of the composition are passed through a "Wiley" hammer mill, wherein the particles are comminuted to a maximum particle size of approximately 5 mesh. The particle size of the pulverized material is controlled by the size of the openings in a screen surrounding the pulverizing chamber. The pulverized material is placed in a mold cavity having an arcuate longitudinal cross section, and a molding  $\frac{1}{16}$ - $\frac{1}{16}$  inch in thickness,  $2\frac{1}{2}$  inches wide, and 5 inches arc length on a 7-inch radius, is obtained by molding at  $360^{\circ}$  F. and 4000 pounds per square inch pressure for a period of one hour. At the end of this time, the mold is cooled to  $150^{\circ}$  F. and the molded article removed from the mold cavity, placed in a "curing" mold having cavity contours of the same general shape as that of the cavity employed in the initial molding operation, and "cured" for a period of 16 hours at  $500^{\circ}$ - $525^{\circ}$  F. The cured molding is cooled to room temperature and fixed to a brake shoe as a brake lining element of a small laboratory dynamometer for testing.

The dynamometer comprises a rear brake assembly of an "International K-5" truck equipped with International Harvester 14-inch diameter brake drums No. 95,223H at each end of the flywheel shaft. The dynamometer is so driven as to simulate the energy effect (94,250 foot pounds) on one wheel of a 10-ton truck in decelerating from a speed of 45 miles per hour to a position of rest in 6 seconds. The cycle frequency from acceleration from a position of rest to top speed, braking to decelerate to a position of rest, and accelerating again is 35 seconds, except during periods for the removal of brake linings for wear measurements, etc. After 10-15 35-second cycles, the brake drum temperature of the brake assembly generally reaches  $400^{\circ}$ - $550^{\circ}$  F., occasionally as high as  $650^{\circ}$  F.; good evidence exists that the actual surface temperature of the lining may go as high as  $1400^{\circ}$  F.

The coefficient of friction  $m$  in this and the other examples hereinafter is calculated from the formula:

$$m = \frac{F}{5.52P + 0.84F}$$

wherein

$F$ =tangential friction force  
 $P$ =load on the brake shoe

and the constants are derived from other formulae developed by analysis of brake members for the particular dynamometer assembly.

The coefficients of friction noted in this and the following examples are calculated from data taken during deceleration in a cycle or series of cycles, whereas the drum temperatures corresponding to these coefficients of friction are

taken before the acceleration in a cycle or averaged at such times over a series of cycles, because of the wide temperature fluctuations occurring during the deceleration of the dynamometer load. The temperatures noted in the results given below therefore represent minimum rather than maximum or average drum temperatures during a given cycle.

#### Test results

The calculated rate of wear per thousand cycles based on 147 cycles is 0.052 inch.

#### FRICITION CHARACTERISTICS

| Brake Drum Temperature, ° F. | Coefficient of Friction |
|------------------------------|-------------------------|
| Room Temperature.....        | 0.40                    |
| 425.....                     | 0.37                    |
| 635.....                     | 0.38                    |

#### EXAMPLE 2

##### Formulation

216 parts of lead sulfate (approximately 300 mesh).

273 parts of a 61.5% solution in isopropyl ether of the co-hydrolyzate of 80 mol per cent of phenyl silicon trichloride and 20 mol per cent of ethyl silicon trichloride, containing 1.6 parts of triethanolamine (condensation catalyst for the cohydrolyzate).

424 parts of asbestos fibers (of the same grade as that used in Example 1).

##### Procedure

These ingredients are mixed together in precisely the same manner as that described for the composition of Example 1 and a molded brake lining element obtained from this composition.

##### Test results

The calculated rate of wear per thousand cycles based on 115 cycles is 0.68 inch.

#### FRICITION CHARACTERISTICS

| Brake Drum Temperature, ° F. | Coefficient of Friction |
|------------------------------|-------------------------|
| Room Temperature.....        | 0.55                    |
| 395.....                     | 0.40                    |
| 605.....                     | 0.32                    |

#### EXAMPLE 3

##### Formulation

425 parts of basic lead sulfate ( $PbSO_4 \cdot PbO$ ) (approximately 300 mesh).

260 parts of a 61.5% solution in isopropyl ether of the co-hydrolyzate of 80 mol per cent of phenyl silicon trichloride and 20 mol per cent of ethyl silicon trichloride, containing 1.6 parts of triethanolamine (condensation catalyst for the organo-silicon chloride co-hydrolyzate).

216 parts of asbestos fibers (of the same grade as that used in Example 1).

##### Procedure

The method of combining these materials and obtaining a molded friction element therefrom is carried out in precisely the same manner as that described in Example 1 above.

##### Test results

The calculated rate of wear per thousand cycles based on 352 cycles is 0.17 inch.

#### FRICITION CHARACTERISTICS

| Brake Drum Temperature, ° F. | Coefficient of Friction |
|------------------------------|-------------------------|
| Room Temperature.....        | 0.40                    |
| 425.....                     | 0.37                    |
| 635.....                     | 0.38                    |

#### EXAMPLE 4

##### Formulation

244 parts of lead sulfate (approximately 300 mesh).

180 parts of lead monoxide (approximately 300 mesh).

260 parts of a 61.5% solution in isopropyl ether of the co-hydrolyzate of 80 mol per cent of phenyl silicon trichloride and 20 mol per cent of ethyl silicon trichloride, containing 1.6 parts of triethanolamine (condensation catalyst for the organo-silicon trihalide co-hydrolyzate).

216 parts of asbestos fibers (of the same grade as that used in Example 1).

##### Procedure

The ingredients of this formula are combined in precisely the same manner as that described in Example 1 and the method of obtaining a molded friction element as described in Example 1 is also employed.

##### Test results

The calculated rate of wear per thousand cycles based on 800 cycles is 0.012 inch.

#### FRICITION CHARACTERISTICS

| Brake Drum Temperature, ° F. | Coefficient of Friction |
|------------------------------|-------------------------|
| Room Temperature.....        | 0.34                    |
| 500.....                     | 0.48                    |
| 635.....                     | 0.45                    |

#### EXAMPLE 5

##### Formulation

##### "A"

76.5 parts of the dry comminuted partially condensed co-hydrolyzate of a mixture of 80 mol per cent of phenyl silicon trichloride and 20 mol per cent of ethyl silicon trichloride.

25.5 parts of the butadiene-acrylonitrile elastomeric copolymer available under the trade-name "Hycar."

0.6 part sulfur.

##### Procedure

The butadiene-acrylonitrile copolymer is milled on a rubber mill having a roll speed differential of 2-3 until a substantially continuous sheet thereof is obtained. The milling of the butadiene-acrylonitrile copolymer is continued and the 76.5 parts of the partially condensed co-hydrolyzate added thereto and the milling continued until a substantially uniform mixture is obtained, after which the sulfur is added as a curing catalyst for the butadiene-acrylonitrile elastomer. Thereafter, the mix is removed from the rubber mill as a substantially continuous sheet, which is cooled by means of dry ice to a temperature at which the mass becomes brittle

and readily friable. The cold brittle mass is placed in a "Wiley" hammer mill and comminuted to a maximum particle size of approximately 5 mesh.

*Formulation*

"B"

168 parts of lead sulfate (approximately 300 mesh).

132 parts of lead oxide (approximately 300 mesh).

198 parts of asbestos fibers (of the same grade as that used in Example 1).

*Procedure*

The lead sulfate-lead monoxide and asbestos fibers are placed in a "Day" mixer and mixed together in the manner described in Example 1 above until a substantially uniform mixture has been obtained, after which the comminuted resinous mixture of "Hycar," partially condensed siloxane resins, and triethanolamine is added to the batch during the mixing operation and the mixing continued until the mixture is uniform. Methyl ethyl ketone in an amount sufficient to wet the entire mass and render it plastic is added during the mixing operation in order substantially to coat all of the particles of the dry inorganic materials with a solution of the resinous material. Thereafter, the solvent is driven from the batch in a manner described in Example 1 and the pulverulent mass thus obtained comminuted in a "Wiley" hammer mill to a maximum particle size of approximately 5 mesh, from which comminuted mass a friction element is obtained by molding in accordance with the technique described in Example 1.

*Test results*

The calculated rate of wear per thousand cycles based on 2000 cycles is 0.0068 inch.

**FRICTION CHARACTERISTICS**

| Brake Drum Temperature, ° F. | Coefficient of Friction |
|------------------------------|-------------------------|
| Room Temperature.....        | 0.31                    |
| 425.....                     | 0.47                    |
| 500.....                     | 0.60                    |
| 590.....                     | 0.55                    |

**EXAMPLE 6**

*Formulation*

"A"

90 parts of the co-hydrolyzate of 80 mol per cent of phenyl silicon trichloride and 20 mol per cent of ethyl silicon trichloride, containing 0.9 part of triethanolamine (condensation catalyst for the co-hydrolyzate).

30 parts of a butadiene-acrylonitrile elastomeric copolymer commercially available under the trade-name of "Hycar."

0.75 part sulfur.

*Formulation*

"B"

168 parts of lead sulfate (approximately 300 mesh).

132 parts of lead monoxide (approximately 300 mesh).

180 parts of asbestos fibers (of the same grade as that used in Example 1).

*Procedure*

Precisely the same procedure as that described in Example 5 is followed in this example to obtain a molded friction element.

*Test results*

The calculated rate of wear per thousand cycles based on 2100 cycles is 0.005 inch.

**FRICTION CHARACTERISTICS**

| Brake Drum Temperature, ° F. | Coefficient of Friction |
|------------------------------|-------------------------|
| Room Temperature.....        | 0.36                    |
| 400.....                     | 0.48                    |
| 475.....                     | 0.60                    |
| 600.....                     | 0.45                    |

**EXAMPLE 7**

*Formulation*

"A"

76.5 parts of the co-hydrolyzate of 80 mol per cent of phenyl silicon trichloride and 20 mol per cent of ethyl silicon trichloride, containing 0.6 part of triethanolamine (condensation catalyst for the co-hydrolyzate material).

25.5 parts of the butadiene-acrylonitrile elastomeric copolymer commercially available under the trade-name of "Hycar."

0.6 part sulfur.

*Formulation*

"B"

35 174 parts of lead sulfate (approximately 300 mesh).

132 parts of lead monoxide (approximately 300 mesh).

40 180 parts of asbestos fibers (of the same grade as that used in Example 1).

12 parts graphite.

*Procedure*

A cured friction element is obtained in precisely the same manner as that described in Example 5 above.

*Test results*

The calculated rate of wear per thousand cycles based on 2000 cycles is 0.007 inch.

**FRICTION CHARACTERISTICS**

| Brake Drum Temperature, ° F. | Coefficient of Friction |
|------------------------------|-------------------------|
| Room Temperature.....        | 0.27                    |
| 420.....                     | 0.50                    |
| 600.....                     | 0.47                    |

**EXAMPLE 8**

*Formulation*

65 60 parts of a co-hydrolyzate of 80 mol per cent of phenyl silicon trichloride and 20 mol per cent of ethyl silicon trichloride, containing 0.6 part of triethanolamine (condensation catalyst for the co-hydrolyzate).

20 parts of the butadiene-acrylonitrile copolymer commercially available under the trade-name of "Hycar."

100 parts of lead sulfate (approximately 300 mesh).

80 parts of lead monoxide (approximately 300 mesh).

7.6 parts of graphite.  
1 part sulfur.

*Procedure*

The organo-silicon trihalide co-hydrolyzate and the "Hycar" are dissolved in 400 mls. of methyl ethyl ketone and the solution placed in a vessel having a propeller agitator inserted through a liquid-tight bearing at the bottom thereof. The agitator is set in motion and the combination of lead sulfate-lead monoxide, graphite, and sulfur are added to the agitated solution in small increments over a period of approximately 10 minutes, after which an additional 50 mls. of methyl ethyl ketone are added. 205 grams of asbestos cloth in the form of 18 strips, 2 inches by 5 inches, are dipped into the agitated suspension, removed therefrom, dried and dipped a second time, removed and dried. The gain in weight of the 18 strips is 185 grams. The resin impregnated strips are assembled in the form of a lamination and placed in the mold described in Example 1 and molded and cured in the manner described in Example 1. The molding thus obtained is placed in the laboratory dynamometer described in Example 1.

*Test results*

The calculated rate of wear per thousand cycles based on 10,000 cycles is 0.0072 inch.

**FRICITION CHARACTERISTICS**

| Brake Drum Temperature, °F. | Coefficient of Friction |    |
|-----------------------------|-------------------------|----|
| Room Temperature.....       | 0.57                    | 35 |
| 550.....                    | 0.40                    |    |

*Discussion of results*

It will be observed from the above examples that when lead monoxide is used in combination with the siloxane material and asbestos (Example 1), the friction element obtained therefrom exhibits an increase in the coefficient of friction with increase of temperature, whereas the composition containing lead sulfate in combination with the siloxane material and asbestos (Example 2) exhibits a decrease in the coefficient of friction with increase of temperature, and that basic lead sulfate ( $PbSO_4 \cdot PbO$ ) in the combination (Example 3) gives a substantially constant coefficient of friction over a wide range of temperatures. However, it will also be observed that in all three of these compositions, the calculated rate of wear per thousand stops is too high for a commercially acceptable friction element.

A comparison of the formulations and the test data of Examples 4-8, all of which include physical mixtures of lead oxide and lead sulfate, show that the combination of a co-hydrolyzate of a phenyl silicon trihalide and an ethyl silicon trihalide with asbestos and a mixture of lead sulfate and lead monoxide in a molded friction element possesses greater wear resistance, heat stability, and a more constant coefficient of friction over a wide temperature range than do similar combinations containing lead sulfate without lead monoxide, or lead monoxide without lead sulfate, or those containing basic lead sulfate ( $PbO \cdot PbSO_4$ ).

A further comparison may be made of the test data given in Examples 4-8, inclusive, with data obtained from commercial brake linings functioning in the same dynamometer as that used in the above examples, and under substantially

the same conditions, by referring to the data set forth in the table below:

| Commercial Truck Lining | Calculated Rate of Wear/1000 Cycles | Based on X Cycles | Coefficient of Friction | At T °F. |
|-------------------------|-------------------------------------|-------------------|-------------------------|----------|
| I.....                  | 0.036                               | 1,125             | 0.00                    | 577      |
| II.....                 | 0.012                               | 396               | 0.00                    | 600      |
| III.....                | 0.023                               | 2,000             | 0.02                    | 480      |
| IV (Heavy Duty).....    | 0.01                                | 812               | -0.23                   | 525      |
| V (Heavy Duty).....     | 0.01                                | 10,000            | -0.11                   | 525      |

These data clearly show the superiority of the compositions of the present invention over commercially available brake linings, particularly in respect to the rate of wear and the coefficient of friction at sustained high temperatures. Commercial brake linings initially exhibit a relatively high coefficient of friction at low temperatures, which rapidly diminish, as shown by the above table of data, in some instances to zero at sustained high temperatures, while friction elements manufactured from the compositions of the present invention exhibit the inverse of this behavior in that the friction elements made therefrom exhibit an increase in the coefficient of friction with increasing temperature to a maximum, after which at sustained high temperatures the coefficient remains substantially constant at a value greater than that exhibited by prior art friction element compositions at low temperatures.

Also of importance to the compositions of the present invention, although somewhat less dramatically demonstrable, is the extended transient thermoplastic range of the particular co-hydrolyzates employed herein. Thus, co-hydrolyzates of a mixture of 70-90 mol per cent of a phenyl silicon trihalide and 10-30 mol per cent of an ethyl silicon trihalide are eminently suited to the manufacture of pressure molded friction elements, especially since they are characterized by remaining fluid throughout the pressure molding operation. This is true whether they are recovered from the hydrolysis reaction mass as a solution and then compounded with the other ingredients of the composition or whether they are recovered as pulverulent solids from such solutions by evaporation of the solvent and subsequently compounded. Thereafter, the co-hydrolyzate material may be "set" or "cured" in a relatively short time and at moderate temperatures to a hard cohesive infusible bond between the particles and fibers of the inorganic portion of the compositions.

While there have been described various embodiments of the invention, the methods and products described are not intended to be understood as limiting the scope of the invention as it is realized that changes therewithin are possible and it is further intended that each element recited in any of the following claims is to be understood as referring to all equivalent elements for accomplishing substantially the same results in substantially the same or equivalent manner, it being intended to cover the invention broadly in whatever form its principle may be utilized.

What is claimed is:

1. A composition of matter, the principal ingredients of which are asbestos, a co-hydrolyzate of a mixture of 10-30 mol per cent of an ethyl silicon trihalide and 70-90 mol per cent of a phenyl silicon trihalide, and a physical mixture of  $PbSO_4$  and  $PbO$ .

## 11

2. A composition of matter, the principal ingredients of which are asbestos, a co-hydrolyzate of a mixture of 10-30 mol per cent of an ethyl silicon trihalide and 70-90 mol per cent of a phenyl silicon trihalide,  $PbSO_4$ , and  $PbO$ , and the lesser ingredients of which include an elastomeric copolymer of butadiene and acrylonitrile.

3. A composition of matter, the principal ingredients of which are asbestos, a co-hydrolyzate of a mixture of 10-30 mol per cent of an ethyl silicon trihalide and 70-90 mol per cent of a phenyl silicon trihalide,  $PbSO_4$ , and  $PbO$ , and the lesser ingredients of which include graphite.

4. A composition of matter, the principal ingredients of which amount to 90-100% thereof and consist essentially of a co-hydrolyzate of a mixture of 10-30 mol per cent of an ethyl silicon trihalide and 70-90 mol per cent of a phenyl silicon trihalide,  $PbSO_4$ ,  $PbO$ , and asbestos, and the lesser ingredients of which amount to up to 10% thereof and include graphite and an elastomeric copolymer of butadiene and acrylonitrile.

5. A friction element composition comprising 5-25% by weight of a co-hydrolyzate of a mixture of 10-30 mol per cent of an ethyl silicon trihalide and 70-90 mol per cent of a phenyl silicon trihalide, 20-75% by weight of asbestos, 25-60% by weight of a mixture of  $PbSO_4$  and  $PbO$  having a molar ratio of  $PbSO_4:PbO$  within the range of 0.4-1.1:1, and up to 10% by weight of graphite and an elastomeric copolymer of butadiene and acrylonitrile.

6. A friction element composition comprising 5-25% by weight of a co-hydrolyzate of a mixture of about 20 mol per cent of an ethyl silicon trihalide and about 80 mol per cent of a phenyl silicon trihalide, 20-75% by weight of asbestos, 25-60% by weight of a mixture of  $PbSO_4$  and  $PbO$  having a molar ratio of  $PbSO_4:PbO$  within the range of 0.4-1.1:1, and up to 10% by weight of graphite and an elastomeric copolymer of butadiene and acrylonitrile.

7. A friction element composition comprising 10.9% of a co-hydrolyzate of a mixture of about 20 mol per cent of an ethyl silicon trihalide and about 80 mol per cent of a phenyl silicon trihalide, 52.9% of asbestos cloth, 14.5%  $PbO$ , 18.1%  $PbSO_4$  and 3.6% of an elastomeric copolymer of butadiene and acrylonitrile.

## 12

8. The method of making friction elements which includes the steps of dipping asbestos cloth in a slurry of a co-hydrolyzate of a mixture of 10-30 mol per cent of an ethyl silicon trihalide and 70-90 mol per cent of a phenyl silicon trihalide, lead oxide, and lead sulfate in a solvent, drying said cloth, redipping said cloth in said slurry, redrying said cloth, assembling a plurality of said dipped dried clothes into a laminate and molding said laminate to obtain a friction element.

9. The method of making friction elements which includes the steps of impregnating asbestos cloth with a co-hydrolyzate of a mixture of 10-30 mol per cent of an ethyl silicon trihalide and 70-90 mol per cent of a phenyl silicon trihalide, lead oxide, and lead sulfate by dipping said cloth in a mixture of said co-hydrolyzate, said lead oxide, and said lead sulfate in a solvent, drying said cloth, assembling a plurality of said dipped dried clothes into a laminate and molding said laminate to obtain a friction element.

10. The method of making friction elements which includes preparing an intimate physical mixture of lead monoxide, lead sulfate, and asbestos, combining therewith a solution of a co-hydrolyzate of a mixture of 10-30 mol per cent of an ethyl silicon trihalide and 70-90 mol per cent of a phenyl silicon trihalide in a solvent, mixing until substantial uniformity is obtained, while evaporating the solvent, placing said material in a mold cavity and molding said material under heat and pressure.

35

JULIUS E. UNDERWOOD.  
ALFRED HIRSCH.

## REFERENCES CITED

The following references are of record in the file of this patent:

## UNITED STATES PATENTS

|              |       |              |
|--------------|-------|--------------|
| Number       | Name  | Date         |
| 45 2,410,737 | Jenny | Nov. 5, 1946 |

## FOREIGN PATENTS

|         |               |              |
|---------|---------------|--------------|
| Number  | Country       | Date         |
| 609,609 | Great Britain | Oct. 5, 1948 |